

## UNITED STATES PATENT OFFICE.

PERCY A. E. ARMSTRONG, OF LOUDONVILLE, NEW YORK.

## ELECTRICAL HEATING ELEMENT.

No Drawing. Application filed December 13, 1919, Serial No. 344,737. Renewed November 24, 1922.

To all whom it may concern:

Be it known that I, PERCY A. E. ARMSTRONG, a subject of the King of Great Britain, and a resident of Loudonville, county 5 of Albany, and State of New York, have invented certain new and useful Improvements in Electrical Heating Elements, of which the following is a specification.

My invention relates to electrical heating 10 elements of alloy steel containing essentially iron, chromium, silicon, aluminum and carbon.

Heating elements in accordance with my 15 invention may contain chromium from about 3% to 30%, silicon from about .5% to about 5%, aluminum from about .4% to about 4%, carbon from about .05% to about 1.5% and preferably under about .50%, and the principal part of the remainder iron.

20 More or less of the metalloids, such as sulphur and phosphorus, may be present, but the same are preferably kept low. Manganese may be present in the usual proportions encountered in steel making, say 25 up to about .85%, but manganese may be dispensed with, if desired.

Relatively cheap electrical heating elements, which are not required to withstand 30 temperatures over about 1300° F., may contain as little as about 3% of chromium, about 1% of silicon, about .5% of aluminum, carbon preferably from about .05% to about .5% and the principal part of the remainder iron. This analysis represents about the 35 minimum proportions of the different materials to give a fair amount of electrical resistance and a good degree of resistance to hot oxidation.

A good example of an element to withstand 40 temperatures up to about 1700° F. is, chromium about 10%, silicon about 3%, aluminum about 3% and carbon about .05% to about 50%.

Another element which gives good results 45 at about the last named temperatures contains chromium about 10%, silicon about 12%, aluminum about 1%, and carbon as before. With the higher content of silicon and aluminum, taken together, increased specific resistance is obtained. With the alloy last described, and having the content

of silicon and aluminum relatively low, a larger wire can be employed which is better adapted for more rugged applications where size and strength are important requirements. 55

A good example of an element to withstand higher temperatures, say up to about 2000° F. to 2200° F., contains chromium about 16%, silicon about 3%, aluminum about .45% and carbon about .05% to about .50%. Elements of this analysis having about .24% of carbon were found to have a specific resistance of 143 microhms per cubic centimeter and desirably long life. 65

One of the beneficial effects of aluminum used in conjunction with silicon is that high specific resistance can be obtained without the use of an unduly large quantity of alloying constituents, making a material 70 which can be mechanically worked to good advantage. Aluminum when used as described, appears to have the valuable property of either holding the gases in solution or taking the oxygen out of the alloy steel. 75 With too great a percentage of aluminum, however, the material is both hot and cold short, but with relatively low amounts of aluminum added, about as stated, the combination of iron, chromium, silicon and carbon is materially improved and better results obtained. Under these circumstances I have found that in my electrical heating elements 80 of alloy steel, silicon and aluminum are not interchangeable, one for the other, but must be used together to get good results. The effect of small quantities of aluminum is most marked in the case of elements for 85 withstanding high temperatures given above. Here the aluminum shown in the analysis of the finished material is but .45%, yet with the same chromium, silicon and carbon, but without aluminum, nowhere near as satisfactory results are obtained. With the use

90 of aluminum as described, a very thin and resistant scale appears to be quickly formed on the surface of the element when subjected to heat and to oxidizing agencies and this skin coating effectively resists further oxidation and scaling in use at high temperatures. 100

I have found that by using carbon under

1.5% and preferably under .5%, I can use a much cheaper grade of material than without the use of carbon. The carbon has a desirable property of refining the grain and preventing undue grain growth under conditions of use, it appears to increase the specific resistance to some extent, it causes the material to flow or conform well to groove shapes in rolling, hastens solidification of the melt, and cuts down the plastic range enabling the elimination of hollow or spongy centers, improves the annealing properties, and imparts a degree of stiffness to the heating elements which is particularly desirable in lateral applications.

Where the elements are made by hot working, as by rolling hot, the carbon content can be increased up to about 1.5%, but for elements made by cold working as by cold drawing into wire the carbon content is preferably under .50% and may be as low as .05%.

Proportions given herein are by weight. It will be understood that more or less variation from the proportions stated can be resorted to, if desired, without departing from

my invention or sacrificing the advantages thereof.

I claim:

1. An electrical heating element made of alloy steel containing chromium about 3% to about 30%, silicon about .5% to about 5%, aluminum about .4% to about 4%, carbon about .05% to about 1.5%, and the principal portion of the remainder iron. 30

2. An electrical heating element made of alloy steel containing chromium about 10% to about 20%, aluminum about .4% to about 4%, silicon about 1% to about 5% and more silicon than aluminum, carbon about .05% to about .50% and the principal part of the remainder iron. 35

3. An electrical heating element of alloy steel containing chromium about 16%, silicon about 3%, aluminum about .45%, carbon under .50%, and the principal portion of the remainder iron. 40 45

In testimony that I claim the foregoing, I hereto set my hand, this 29th day of November, 1919.

PERCY A. E. ARMSTRONG.